

# United States Patent

[11] 3,597,886

[72] Inventors **Vladimir Vasilievich Sapozhnikov**  
Petropavloskaya ulitsa, 8, kv. 10;  
**Vladimir Nikolaevich Smirnov**, ulitsa  
Smirnova, 13, kv. 27; **Alexandr**  
Mikhailovich Solov'ev, Prospekt Smirnova,  
13, kv. 60; **Roman Izrailevich Shneider**,  
ulitsa Plekhanova, 16, kv. 12, all of  
Leningrad, U.S.S.R.

[21] Appl. No. **806,725**

[22] Filed **Mar. 12, 1969**

[45] Patented **Aug. 10, 1971**

[54] **METHOD OF VIBROABRASION TREATMENT OF**  
**SMALL-SIZED PARTS**  
5 Claims, No Drawings

[52] U.S. Cl. .... **51/316**

[51] Int. Cl. .... **B24b 1/00**

[50] **Field of Search** .... **51/313,**  
**314, 315, 316, 317, 7, 164.5**

[56] **References Cited**  
UNITED STATES PATENTS  
389,552 9/1888 **Dean** ..... **51/164.5**

957,999 5/1910 Parsons ..... **51/164.5 X**  
1,017,268 2/1912 Parsons ..... **51/316**  
3,187,473 6/1965 Ruppe ..... **51/313**

*Primary Examiner*—Lester M. Swingle  
*Attorney*—Waters, Roditi, Schwartz & Nissen

**ABSTRACT:** According to the method proposed herein, in an inert liquid medium are introduced abrasive powder and metallic bodies or particles which are capable of fixing the particles of abrasive powder on their surface and grinding these while interacting with said abrasive powder in the course of treatment of the small-sized parts involved, said abrasive powder that is introduced into said inert liquid medium, should feature its granularity permissible to perform the initial stage of treatment of the small-sized parts involved e.g. coarse grinding, whereas the quantitative ratio between the metallic bodies and abrasive powder that are introduced into said liquid medium, must be so selected as to provide a successive and complete grinding of abrasive powder till obtaining its granularity necessary to perform the final stage of treatment of said small-sized parts e.g. buffing.

## METHOD OF VIBROABRASION TREATMENT OF SMALL-SIZED PARTS

The present invention relates to methods of vibroabrasion treatment of small-sized parts, mainly for precision instruments that have friction surfaces whose finish should conform to the highest quality grades.

Widely known in the art is a method of vibroabrasion treatment of small-sized parts with abrasive powder in an inert liquid medium.

The above-said method, however, suffers from numerous substantial disadvantages such as: low productivity; repetitive operations of the method due to the fact that a coarse-grained abrasive powder must be employed at the initial stage of the grinding process and a fine-grained powder must be employed at the final stage thereof; the necessity for use of high-dispersive homogeneously grained abrasive powders at the final stage of treatment; impossibility to obtain surfaces finished to a quality that should meet high requirements specified for a variety of components made use of in precision instruments such as pivots of electric measuring instruments; and the fact that in treating parts the stock is removed mostly from protruding parts thereof.

Another method of vibrotreatment is in an inert liquid medium with the use of abradant-bearing filling agents.

This method though more productive, suffers from all the disadvantages inherent in the method of vibrotreatment with abrasive powder and, moreover, involves the use of specially prepared filling agent.

It is an object of the present invention to eliminate the disadvantages mentioned above.

It is the main object of the present invention to provide a method of vibrotreatment of small-sized parts, whereby said parts pass uninterruptedly through all the process stages at one cycle, starting from the coarse and up to the finest one (coarse grinding, fine grinding, buffing), with the possibility to vary the amount of the stock removed and the rate of its removal from the protruding parts.

Said object is accomplished due to the fact that in an inert liquid medium are introduced abrasive powder and metallic bodies, said bodies being capable, while interacting with abrasive powder in the course of treatment of small-sized parts, of fixing abrasive powder particles on their surface and grinding them. It is expedient that abrasive powder introduced into an inert liquid medium, feature its granularity to perform the initial stage of treatment of small-sized parts, e.g. coarse grinding, whereas the quantitative ratio between the metallic bodies and abrasive powder that are introduced into a liquid medium, must be so selected as to provide a successive and complete grinding of abrasive powder obtaining the granularity necessary to perform the final stage of treatment, e.g. buffing.

High-tin bronze can be made use of as the material of the aforementioned metallic bodies capable of fixing the particles of abrasive powder on their surface to grind them.

Both abrasive powder and the metallic bodies capable of fixing the abrasive powder particles on the surface thereof, are introduced into an inert liquid medium constituted by at least two fluids different in viscosity.

The method disclosed herein allow the performance of an entire cycle of treatment (i.e. coarse grinding, fine grinding, polishing, polishing and buffing) without changing the inert liquid medium, abrasive powder and metallic bodies capable of fixing the abrasive powder particles on the surface thereof, since in the course of treatment, successively decreasing particles of abrasive powder are fixed on the metallic bodies.

The method in question makes it possible to vary the rate of removal and the amount of the stock removed from the protruding portions of the parts being treated, by varying the ratio between the differently viscous fluids constituting the inert liquid medium involved.

The herein-proposed method prevents foreign objects from contacting the surface of the parts being treated thus eliminat-

ing possible adverse effect of said objects upon the quality of surface finish obtained.

The present method does not involve the use of high-dispersive abrasive powders, inasmuch as the latter are formed as a result of grinding larger grains of the initially introduced abrasive powder.

According to the herein-considered method, in the course of treatment of parts their superficial strengthening simultaneously occurs.

The application of the method of the present invention reduces the expenses for treatment of parts due to a simplified technological process and a low cost of the raw materials used.

To promote understanding a few examples of vibrotreatment of small-sized parts by the method disclosed herein, are described hereinbelow.

### EXAMPLE 1

Treatment of carbon-steel blanks of pivots for electric measuring instruments is involved, the length of a blank being equal to 3 mm. and its diameter equal to 0.5 mm. The blanks are to be treated until a fillet radius of 35 microns is obtained, with simultaneous grinding, polishing and buffing of the blank tapered portion.

In a container holding 10 cc. of an inert fluid constituted by 9 cc. of kerosene and 1 cc. of bone oil, are introduced 300 mg. of abrasive powder 25 grams of 1.3 mm. diameter globules or pellets made of high-tin bronze, and 1000 blanks of pivots.

This done, the above-mentioned container is imparted oscillating motion at a frequency of 50 c./s. and an amplitude of 4 mm. In 25 hours the treatment cycle is completed.

Then the inert fluid is drained off, whereas a mixture of parts and globules is rinsed in gasoline and dried. Next the finished pivots are separated out from the globules by sieving through a rectangular-mesh screen. The globules are employed for treating fresh lots of parts.

The fillet radius of the finished pivots equals 35 microns, the quality of surface finish on both the tapered portion and the fillet of pivots being in compliance with the highest quality grades. No traces of treatment are found on the finished surface when investigated under a microscope of a 120<sup>x</sup> magnification. Moreover, the finished pivots when used in electric measuring instruments, feature their abrasion-resistance under a vibratory load 1.5 times as high as compared to those treated by any other methods, this being due to the fact that they have been given additional superficial strengthening in the course of treatment.

### EXAMPLE 2

Treatment of carbon-steel blanks of pivots for electric measuring instruments is involved, the length of a blank equaling 3 mm. and its diameter 0.5 mm. The blanks are to be treated until a fillet radius of 20 microns is obtained, with simultaneous grinding, polishing and buffing of the blank tapered portion.

In a container holding 10 cc. of an inert fluid composed of 8 cc. of kerosene and 2 cc. of bone oil, are introduced 120 mg. of abrasive powder, 15 grams of 1 mm. diameter globules or pellets made of high-tin bronze, and 1000 blanks of pivots.

Thereupon the container is imparted oscillating motion at a frequency of 50 c./s. and an amplitude of 4 mm. The treatment cycle is to take a period of 20 hrs., whereupon the inert fluid is drained off and a mixture of parts and globules is washed in gasoline and dried.

Then the finished pivots are separated out from the globules by sieving through a rectangular-mesh screen, whereafter the globules are ready to be used for treating fresh lots of parts. The fillet radius of the finished pivots equals 20 microns, the quality of surface finish on both the tapered portion and the fillet of pivots is found to meet the highest quality grades. No traces of treatment are revealed on the finished surface when investigated under a 120<sup>x</sup>-magnification microscope. Like in the above-stated example, superficial strengthening of the parts takes place.

## EXAMPLE 3

Treatment of carbon-steel blanks of trunnions for measuring gears of electric measuring instruments is involved, the length of the effective portion of a blank being equal to 1 mm. and its diameter equal to 0.5 mm.

In a container which holds 10 cc. of an inert fluid composed of 9.5 cc. of kerosene and 0.5 cc. of bone oil, are introduced 200 mg. of abrasive powder, 20 grams of 1.2 mm. diameter globules or pellets made of high-tin bronze, and 500 parts to be treated.

Then the container is imparted oscillating motion at a frequency of 50 c./s. and an amplitude of 4 mm. Once the 40 hr. working cycle has been completed, the inert fluid is drained off and a mixture of parts and globules is rinsed in gasoline and dried.

The finished trunnions are separated out from the globules by sieving through a screen having its meshes shaped to suit the shape of the finished trunnions, while the globules are ready to be employed for treating fresh lots of parts. The finished trunnions feature the quality of surface finish on the effective portion thereof as to comply with the highest quality grades. No traces of treatment are found on the finished surface when investigated under a 120<sup>x</sup>-magnification microscope. Similar to the examples 1 and 2 above, a superficial strengthening of the parts occurs.

What we claim is:

1. A method of vibroabrasion treatment of small-sized parts in an inert liquid medium, comprising introducing into said inert liquid medium abrasive powder and metallic bodies in a predetermined ratio, said metallic bodies being constituted so

as to be capable of fixing the abrasive powder particles on their surface and grinding them while interacting with said abrasive powder in the course of treatment of the small-sized parts involved, and vibrating said inert liquid medium together with the small-sized parts under treatment, and abrasive powder and metallic bodies immersed therein.

2. A method of vibroabrasion treatment of small-sized parts in an inert liquid medium as claimed in claim 1, in which the abrasive powder introduced into the inert liquid medium, is constituted such that its granularity effects the initial coarse grinding stage of treatment of the small-sized parts involved, the quantitative ratio between the metallic bodies and abrasive powder that are introduced into said inert liquid medium being such so as to provide a successive and complete grinding of the abrasive powder until obtaining the granularity necessary to perform the final buffering stage of treating said small-sized parts.

3. A method of vibroabrasion treatment of small-sized parts in an inert liquid medium as claimed in claim 1, in which introduced into said inert liquid medium are the metallic bodies which are constituted of high-tin bronze.

4. A method of vibroabrasion treatment of small-sized parts in an inert liquid medium as claimed in claim 2, in which introduced into said inert liquid medium are the metallic bodies which are constituted of high-tin bronze.

5. A method of vibroabrasion treatment of small-sized parts in an inert liquid medium as claimed in claim 1, in which the abrasive powder and metallic bodies are introduced into the medium constituted of at least two fluids different in viscosity.

30

35

40

45

50

55

60

65

70

75